# EUROPEAN PATENT SPECIFICATION

(11) **EP 0 219 157 B1**
(45) Date of publication and mention of the grant of the patent: **31.01.1990**
(21) Application number: 86201679.7
(22) Date of filing: 29.09.1986
(51) Int. Cl.: C25C 3/28, C25C 3/00

(54) **Process for the electrolytic production of metals**
Verfahren zur elektrolytischen Herstellung von Metallen
Procédé de production électrolytique de métaux

(30) Priority: 02.10.1985 NL 8502687
(43) Date of publication of application: 22.04.1987
(73) Proprietor: SHELL INTERNATIONALE RESEARCH MAATSCHAPPIJ B.V., 2596 HR Den Haag (NL)
(72) Inventor: Warren, Geoffry Frank, Bogoto (CO); Horstik, Alfred, NL-6827 AT Arnhem (NL); Corbetta, Alberto, NL-2262 AV Leidschendam (NL); Malpas, Richard Edward, Nr. Chester Cheshire (GB); Honders, Antonie, NL-6827 AT Arnhem (NL); van Eijden, Gerbrand Jozef, NL-6827 AT Arnhem (NL)
(74) Representative: Aalbers, Onno

(56) References cited:
- EP-A- 0 039 873
- DE-B- 1 139 985
- GB-A- 660 908

## Description

The invention relates to a process for the electrolytic production of metals from metal halides in the presence of a salt melt of one or more alkali metal or alkaline earth metal halides, in particular chlorides, an example thereof being production of titanium from titanium tetrachloride.

Winning metals by electrolysis in the presence of molten salts is an area in which increasing research is being carried out. An embodiment of this process is known from US-A 2 757 135. In this event titanium tetrachloride is supplied to the electrolysis cell by introducing into the salt melt. In practice, that process has to be carried out with a diaphragm that prevents the flow of titanium in lower valencies to the anode. If this were not done, the titanium would be re-oxidized at the anode to tetravalent titanium and would thus give rise to a loss of current and raw material. Furthermore, the build-up of titanium in the diaphragm shortens its life, which is a significant disadvantage.

The present invention proposes a process for the production of metals Me by electrolysis in the presence of a salt melt of one or more alkali metal or alkaline earth metal halides without using any bipolar electrode which comprises introducing a metal halide MeXn into a cathode consisting of a molten metal M or a molten alloy M.Meₓ, in which Me represents a metal selected from Ti, Hf, Ta, AI, Zr, W, Nb, V, Mo, In, and Ag, M represents a metal selected from Zn, Cd, Sn, Pb, In, Bi and Ga, X represents halogen, n represents the valency of the metal Me and X represents the atomic ratio of Me to M, thus producing an alloy M.Mey in which y represents the atomic ratio of Me to M, y:x being > 1, withdrawing alloy M.Mey from the cathode into which the metal halide was introduced and recovering metal Me from the alloy.

The invention will be discussed in more detail with reference to figures 1 and 2, which illustrate possible electrolytic cells, taking the electrolysis of titanium tetrachloride to produce metallic titanium in a liquid zinc cathode as example.

In Fig. 1 cell 1 is in a jacket of thermally insulating material 2, for example refractory brick. Cathode 3 consists of liquid zinc to which current is fed via insulating pipe 4 and feed rod 4a. Supply of titanium tetrachloride takes place via pipe 5 and distributor 6, for example a metal grid with outlets at intervals or a body of porous ceramic material. Anode 7 is positioned in electrolyte 8 near the interface between cathode and electrolyte. The horizontal surface area of the anode is chosen to be as large as possible. Electrolyte 8, for example a lithium chloride/potassium chloride melt, is heated to a high temperature, for example 350 to 900 _{°}C or higher if operations are carried out under pressure. Through lid 9 runs a supply pipe 10 for inert gas, for example argon, and a discharge pipe 11 for chlorine gas which is generated at the anode. The current and the supply of titanium tetrachloride are adjusted to match each other such that all or substantially all titanium is reduced in the cathode, thus forming a zinc/titanium alloy. This means that the anode does not need to be shielded by a diaphragm. This can be achieved with, for example a current of at least 4 Faraday per mol titanium tetrachloride. Vaporization of titanium tetrachloride before its introduction into the cathode is not necessary, since its temperature rises in any case to above its boiling point (136 _{°}C) during its passage through the salt melt. If desired, the cell can also be provided with means for a correct temperature control of the process. The space above electrolyte 8 can also be cooled or any vaporized salt melt of zinc can be internally or externally condensed and fed back. Supply and discharge of cathode liquid takes place via lines 12 and 13, in particular in the continuous embodiment. The titanium content in the Zn/Ti alloy will be allowed to increase to a predetermined value, preferably between 6 and 20 %wt. Recovery of titanium metal from the alloy may be carried out by conventional methods, e.g. by distilling off cathode metal.

Figure 2 shows a cell with a vertically positioned anode. The same reference numerals have been retained for the same elements of the construction. In the salt melt a tray 14 is placed in which liquid zinc is present. Titanium tetrachloride vapour now enters via perforations in the lower part of supply pipe 5. Anode 7 is constructed as a closed cylinder which completely surrounds the cathode.

Although in the preceding section the process of this invention has been described by reference to the most preferred embodiment, i.e. production of titanium from titanium tetrachloride employing a liquid zinc cathode, the invention is not limited thereto. Analogous processing can be carried out with different cathode materials, i.e. cadmium, tin, lead, bismuth, indium and gallium, from which tin and lead are preferred. Likewise other feedstocks may be processed, i.e. halides of hafnium, tantalum, aluminium, zirconium, tungsten, niobium, vanadium, molybdenum, indium, and silver. Preferred metal halides to be processed are those of tantalum, tungsten, vanadium and niobium. The preferred halogen atom is chlorine, as it is for the molten salt compositions.

It is not known to what extent the production of metal Me proceeds via the direct electrolytic conversion of for example Ti4+ →+ 4e -7 Ti. Introduction of TiC1₄ into a liquid zinc cathode at elevated temperature may result in a chemical reduction of metal Me to lower valencies, for example 2TiCI₄ + Zn -₇ 2TiClε + ZnCi₂, this may then be followed by electrolytic reduction of trivalent titanium to metallic (zerovalent) titanium, coupled with electrolytic regeneration of cathode material by reducing divalent zinc to metallic (zerovalent) zinc. Such combined chemical and electrolytic reductions of metal Me in a higher valency to zerovalent metal are included expressis verbis in the scope of this invention, so is the production of zerovalent tantalum from TaCls in a liquid zinc cathode which probably proceeds entirely via chemical reduction by metallic zinc and electrolytic regeneration (reduction) of cathode material. What is essential to this invention is the application of an electrolytic cell with a liquid metal or alloy cathode, an introduction of metal halide MeXn directly into the liquid cathode and production of (zerovalent) metal Me within the cathode material, the latter as distinguished from production of metal Me somewhere else, i.e. in the molten salt electrolyte or by deposition on a second or auxiliary cathode. Absence of a diaphragm is also important.

The salt melts may be free from impurities but this is not strictly necessary, while in addition it may be advantageous to work under an inert atmosphere of, for example, argon or nitrogen. Examples of suitable salt melts are LiCI/NaCl, NaCI/KCI, LiCI/KCI, LiCl/CaCl₂, NaCl/BaCl₂ and KCI/CaCI₂, but, as has already been pointed out, the invention is not limited to the above-mentioned melts.

In principle, suitable processing temperatures are above the melting point of the cathode material and below the temperature at which that material has such a vapour pressure that undesirably large losses occur. Preferred temperatures are between 400 and 900 °C, for zinc 425 to 890 _{°}C, for cadmium 400 to 700 °C. Similarly, the processing temperature should not be so high that loss of molten salt electrolyte by evaporation or decomposition becomes substantial.

The current and the supply of metal halide feedstock are so adjusted that complete reduction of metal Me in the cathode can take place. Preferably, at least n F.mol-^{I} metal halide MeXₙ is supplied, n being the valency of the metal. The current is, however, restricted to a certain maximum, since deposition of salt-melt metal in the cathode should preferably be prevented as far as possible. The feedstock should preferably be introduced under homogeneous distribution into the cathode. The easiest way for achieving this is by using feedstocks that are in gaseous form on the moment of their introduction into the cathode material. However, introduction into the cathode of compounds in finely dispersed, solid form is also included within the scope of this invention. This all results in no metal Me, or practically none, in any valency ending up in the salt melt. It is then not necessary to employ a diaphragm to shield the anode, so that no undesired current and voltage losses occur, resulting in great technical and economical benefits. Cells having no diaphragm are preferred.

In the alloy M.Mey that is withdrawn from the electrolysis cell y represents the atomic ratio of Me to M. This ratio will usually be kept below 0.5, preferably below 0.3. For easier ways of recovering metal Me from the alloy it is preferred to process alloys in which the content of metal Me is of from 6 to 20 %wt, based on the weight of the alloy.

The invention is elucidated below by a number of experiments.

### Example I

a. 1.5 kg of eutectic LiCI/KCI mixture (59:41 mol) was purified by passing HCI gas through it at above its melting point for 8 hours. The HCI forces the equilibria a) and b) shown below to the left, so that an anhydrous, almost oxygen-free melt is obtained.

Residual oxygen compounds and metallic impurities are then removed by electrolysis under vacuum at a cell voltage of 2.7 V.

An electrolytic cell of externally heated stainless steel was employed with a molten zinc cathode (90 g) which was placed in a holder of A1₂0₃ on the bottom of the cell. A graphite rod served as anode, no diaphragm was used and 250 g salt melt was used as electrolyte. The cell voltage was 5.0 V, the cathode potential was -2.0 V (relative to an Ag/AgCI reference electrode) and the other conditions are given in Table I. The TiC1₄ was injected as a liquid in an argon stream and fed into the cathode. An argon atmosphere was maintained above the salt melt. In all experiments a current of 6 F.mol-¹ TiCI₄ was employed. The following results were determined by microprobe and chemical analysis of the cooled solids.

b. Alloy produced in the first experiment of Table I was subjected to distillation in order to remove all zinc. Upon analysis the remaining residue appeared to consist of very pure titanium.

### Example II

Employing various cathode materials TiCl₄ was electrolysed in the manner described in example la, under the same conditions except those indicated in Table II.

### Example III

Employing various metal halide feedstocks and various cathode materials, experiments were run as described in example I under the same conditions except as those indicated in Table III.

## Claims

1. A process for the production of metals Me by electrolysis in the presence of a salt melt of one or more alkali metal or alkaline earth metal halides without using any bipolar electrode, which comprises introducing a metal halide MeXₙ into a cathode consisting of a molten metal M or a molten alloy M.Meₓ, in which Me represents a metal selected from Ti, Hf, Ta, Al, Zr, W, Nb, V, Mo, In, and Ag, M represents a metal selected from Zn, Cd, Sn, Pb, In, Bi and Ga, X represents halogen, n represents the valency of the metal Me and x represents the atomic ratio of Me to M, thus producing an alloy M.Mey in which y represents the atomic ratio of Me to M, y:x being > 1, withdrawing alloy M.Mey from the cathode into which the metal halide was introduced and recovering metal Me from the alloxy.

2. A process as claimed in claim 1, in which metal halide MeXₙ is distributed in gaseous form through the liquid cathode material.

3. A process as claimed in claim 1 or 2, in which X represents chlorine.

4. A process as claimed in any one of claims 1 to 3, in which the withdrawn alloy comprises 6 to 20 %wt of metal Me, calculated on the weight of the alloy, and in which Me is titanium.

5. A process as claimed in any one of claims 1 to 4, in which a current of at least n F.mol-^{I} is employed, n being the valency of metal Me in the feedstock.

6. A process as claimed in any one of claims 1 to 5, in which the molten salts are chlorides.

7. A process as claimed in any one of claims 1 to 6, in which metal Me is selected from Ti, Ta, W, V and Nb.

8. A process as claimed in claim 7, in which metal Me is Ti.

9. A process as claimed in any one of claims 1 to 8, in which metal M is Zh, Sn or Pb.

10. A process as claimed in claim 9, in which metal M is Zn.

11. A process as claimed in any one of claims 1 to 10, which is carried out in an electrolytic cell having no diaphragm.

## Patentansprüche

1. Ein Verfahren zur Herstellung von Metallen Me durch Elektolyse in Gegenwart einer Salzschmelze eines oder mehrerer Alkalimetall- oder Erdalkalimetallhalogenide ohne Verwendung einer bipolaren Elektrode, welches das Einführen eines Metallhalogenids MeXₙ in eine Kathode, bestehend aus einem geschmolzenen Metall M oder einer geschmolzenen Legierung M.Meₓ, wobei Me ein Metall darstellt, das ausgewählt ist aus Ti, Hf, Ta, Al, Zr, W, Nb, V, Mo, In. und Ag, M ein Metall ist, das ausgewählt ist aus Zn, Cd, Sn, Pb, In, Bi und Ga, X Halogen bedeutet, n die Wertigkeit des Metalls Me ist und x das Atomverhältnis von Me zu M bedeutet, wodurch eine Legierung M.Mey entsteht, in welcher y das Atomverhältnis von Me zu M ist, wobei y:x >1 ist, das Abziehen der Legierung M.Mey aus der Kathode, in welche das Metallhalogenid eingeführt wurde, und das Wiedergewinnen des Metalls Me aus der Legierung umfaßt.

2. Ein Verfahren wie in Anspruch 1 beansprucht, in welchem das Metallhalogenid MeXₙ in gasförmigem Zustand durch das flüssige Kathodenmaterial hindurch verteilt wird.

3. Ein Verfahren wie in Anspruch 1 oder 2 beansprucht, in welchem X Chlor bedeutet.

4. Ein Verfahren wie in einem der Ansprüche 1 bis 3 beansprucht, in welchem die abgezogenen Legierung 6 bis 20 Gewichtsprozent an Metall Me enthält, bezogen auf das Gewicht der Legierung, und in welchem Me Titan ist.

5. Ein Verfahren wie in einem der Ansprüche 1 bis 4 beansprucht, in welchem ein Strom von mindestens n F.mol-¹ angewendet wird, wobei n die Wertigkeit des Metalls Me im Einsatzmaterial ist.

6. Ein Verfahren wie in einem der Ansprüche 1 bis 5 beansprucht, in welchem die geschmolzenen Salze Chloride sind.

7. Ein Verfahren, wie in einem der Ansprüche 1 bis 6 beansprucht, in welchem das Metall Me ausgewählt ist aus Ti, Ta, W, V und Nb.

8. Ein Verfahren, wie in Anspruch 7 beansprucht, in welchem das Metall Me Ti ist.

9. Ein Verfahren wie in einem der Ansprüche 1 bis 8 beansprucht, in welchem das Metall M Zn, Sn oder Pb ist.

10. Ein Verfahren, wie in Anspruch 9 beansprucht, in welchem das Metall M Zn ist.

11. Ein Verfahren wie in einem der Ansprüche 1 bis 10 beansprucht, welches in einer elektrolytischen Zelle ohne Diaphragma durchgeführt wird.

## Revendications

1. Un procédé pour la production de métaux Me par électrolyse en présence d'une masse fondue de sel d'un ou de plus d'un halogénure de métal alcalin ou de métal alcalino-terreux sans utiliser d'électrode bipolaire, qui consiste à introduire un halogénure de métal MeXn dans une cathode constituée d'un métal fondu M ou d'un alliage fondu M.Mex, dans une cathode constituée d'un métal fondu M ou d'un alliage fondu M.Meₓ, dans lequel Me représente un métal choisi parmi Ti, Hf, Ta, AI, Zr, W, Nb, V, Mo, In et Ag, M représente un métal choisi parmi Zn, Cd, Sn, Pb, In, Bi et Ga, X représente de l'halogène, n représente la valence du métal Me et x représente le rapport atomique de Me à M, en produisant ainsi un alliage M.Mey dans lequel y représente le rapport atomique de Me à M, y:x étant supérieur à 1, en éliminant l'alliage M.Mey de la cathode dans laquelle l'halogénure de métal a été introduit et en récupérant le métal Me de l'alliage.

2. Un procédé tel que revendiqué dans la revendication 1, dans lequel l'halogénure de métal MeXₙ est distribué sous une forme gazeuse à travers le matériau liquide de cathode.

3. Un procédé tel que revendiqué dans la revendication 1 ou 2, dans lequel X représente du chlore.

4. Un procédé tel que revendiqué dans l'une quelconque des revendications 1 à 3, dans lequel l'alliage prélevé comprend de 6 à 20% en poids de métal Me, calculé sur le poids de l'alliage, et dans lequel Me est du titane.

5. Un procédé tel que revendiqué dans l'une quelconque des revendications 1 à 4, dans lequel un courant d'au moins n F.mole-¹ est utilisé, n étant la valence du métal Me dans la charge.

6. Un procédé tel que revendiqué dans l'une quelconque des revendications 1 à 5, dans lequel les sels fondus sont des chlorures.

7. Un procédé tel que revendiqué dans l'une quelconque des revendications 1 à 6, dans lequel le métal Me est choisi parmi Ti, Ta, W, V et Nb.

8. Un procédé tel que revendiqué dans la revendication 7, dans lequel le métal Me est Ti.

9. Un procédé tel que revendiqué dans l'une quelconque des revendications 1 à 8, dans lequel le métal M est Zn, Sn ou Pb.

10. Un procédé tel revendiqué dans la revendication 9, dans lequel le métal M est Zn.

11. Un procédé tel que revendiqué dans l'une quelconque des revendications 1 à 10, qui est réalisé dans une cellule électrolytique ne possédant pas de membrane.
